

A. N. DUBOIS.

## PROCESS OF LISLEING AND DYEING VEGETABLE FABRICS.

APPLICATION FILED DEO. 2, 1909.

1,116,397.

Patented Nov. 10, 1914.

2 SHEETS—SHEET 1.



Witnesses:

F. C. Valentine  
T. L. Mockler

*Inventor:*  
*Alexander N. Dubois,*  
*by Obed G. Billman*  
*Attorney.*

A. N. DUBOIS.  
PROCESS OF LISLEING AND DYEING VEGETABLE FABRICS.  
APPLICATION FILED DEO. 2, 1909.

1,116,397.

Patented Nov. 10, 1914.

2 SHEETS—SHEET 2.



Witnesses:

H. C. Valentine  
T. L. Nockton

Fig. 4

Inventor:  
Alexander N. Dubois,  
by Obed C. Billman  
Attorney.

# UNITED STATES PATENT OFFICE.

ALEXANDER N. DUBOIS, OF PHILADELPHIA, PENNSYLVANIA.

## PROCESS OF LISLEING AND DYEING VEGETABLE FABRICS.

1,116,397

Specification of Letters Patent.

Patented Nov. 10, 1914.

Application filed December 2, 1909. Serial No. 530,923.

*To all whom it may concern:*

Be it known that I, ALEXANDER N. DUBOIS, a citizen of the United States, residing at Philadelphia, in the county of Philadelphia, 5 and State of Pennsylvania, with office and laboratory at 835 North Tenth street, Reading, Pennsylvania, have invented certain new and useful Improvements in Processes of Lisleing and Dyeing Vegetable Fabrics, 10 of which the following is a specification.

My invention relates to improvements in a process of lisleing and dyeing vegetable fabrics, particularly cotton goods in the piece, and knitted goods, such as underwear and 15 waists, in the roll.

My invention depends upon my discovery that under certain conditions the treatment of vegetable-fiber fabrics with certain chemicals having the property of disorganizing 20 cellulose fiber may be made use of to act upon and facilitate the removal of the filamental fiber projecting from the surface of the goods without injuriously affecting the body of the goods, and on the contrary with 25 the effect of imparting to it a superior luster and finish, and bringing it to a condition which facilitates the operation and the effect of dyeing.

My invention relates to improvements on 30 the "Process of giving lisle-thread finish to vegetable fabrics", patented to me March 17, 1903, No. 728,147, said process, however, being applicable only to hosiery and knitted garments and entirely impracticable of application to knitted goods in the roll, such 35 as underwear, sweaters and waists, and woven cotton goods in the piece.

It is therefore an object of this invention to provide a process of imparting a lisle-thread finish to such goods, and with this 40 end in view, I employ specially designed machinery herein shown and described.

My invention also relates to an improved process or method of dyeing vegetable fabrics, said process or method being employed 45 in and in conjunction with, the process of lisleing the goods, as well as constituting further steps in the process or method of treatment of the same, as hereinafter 50 described.

Generally speaking, my process or method of treatment consists in,—First: boiling the goods in either plain water, or in alkalized water, according to the results desired, and 55 washing for the purpose of rendering the cotton absorbent to receive the chemical

compound with which it is subsequently treated. Second: extracting the liquid in the goods by means of a hydro-extractor, or a wringer. Third: saturating the goods 60 with a chemical compound adapted to produce the finish desired, said chemical compound having an acid-radical adapted to carbonize the superficial filamental fuzz, and subjecting to heat and attrition until the 65 fuzz is removed and the surface finished. Fourth: washing the goods in a slightly alkaline water whereby the acids left in the goods are neutralized. Fifth: as a part of 70 the dyeing operation instead of the neutralizing treatment just mentioned, giving the goods a special chemical bath adapted to produce a coloration on the goods through the action of the chemical bath in conjunction with the acid left in the goods from the 75 chemical lisleing compound, as hereinafter fully described. Sixth: subjecting the goods so treated to a bleaching bath which may be the ordinary chlorid of lime bleach, the chlorin bleach extracted from rock-salt by 80 electrolysis, the bisulfite or sulfite of soda bleach with permanganate of potash, the sodium peroxid bleach, or the hydrogen peroxid bleach. In any case, the original lisle-thread finish will be preserved and retained 85 in all its beauty.

My process of treatment may take place as a part of the dyeing operation, if the goods are to be dyed, or preparatory to 90 bleaching and dyeing, according to the results desired. There are certain advantages in both methods of treatment as will hereinafter more fully appear.

In actual practice I have applied my process as follows with great success: I first 95 prepare the lisleing compound, this lisleing compound being prepared according to the work to be done, or the results desired. If for cotton cloth in the piece, or knit cotton goods in the roll, such as underwear, sweaters and waists to be bleached or dyed after being given the lisle-thread finish, I make the lisleing compound as follows: For a tub holding 5,000 lbs. of water, I first take about 1000 lbs. of cold water and add to it 100 25 lbs. of ordinary starch. This is stirred up well until the starch is thoroughly dissolved after which the steam valve is opened and the stirring continued to prevent the formation of the starch in lumps, 110 and until the whole is near the boiling point; I then partially shut off the steam

and keep on boiling for about 5 minutes; at the end of this period, I shut off the steam entirely and add to the boiling starch solution either 150 lbs. of ordinary alum, (preferably in powdered form) or 112½ lbs. of granular sulfate of aluminium, and keep stirring until all is well dissolved; I then add cold water to make up the balance of the 5,000 lbs. weight of solution and cool 10 down to about 90° Fahrenheit; I then add from 62½ lbs. to 187½ lbs. commercially pure hydrochloric acid, according to the alkalinity of the water. For example—if the water on analysis gives .05 parts of permanent and .014 parts temporary hardness 15 per 1,000,000 parts water, 62½ lbs. of acid will be proper. If, however, the water has given 0.25 parts temporary hardness the acid required will be about 100 lbs., but if 20 the test has given permanent hardness of 0.18 and 0.40 parts temporary hardness per 1,000,000, per water, then in this case 187½ lbs. of hydrochloric acid will be required to take up the excess of the alkali and permit 25 the slight beginning of carbonization to take place in the goods necessary to produce the desired lisle-thread finish when the goods are subjected to heat and attrition. If desired, the starch in the above de- 30 scribed compound may be omitted and the final result will be the same but the process will be slower. After the goods have been boiled and washed and hydro-extracted as above described, they are then subjected to 35 and saturated with a lisleing compound such as above described for a period of from 15 to 20 minutes, after which they are passed through a hydro-extractor, or passed through a wringer, so as to retain 40 from 50 to 60 lbs. of the lisleing liquid or compound to 100 lbs. (dry weight) of the goods. The liquid that passes through the hydro-extractor is returned to the stock solution in the tub to be used over again. 45 Referring to the drawings, Figure 1, is a side elevation of a machine which I have employed with great success in carrying out my process as applied to knit goods in the roll. Fig. 2, an end elevation of the same. 50 Fig. 3, a top plan view of a machine for the treatment of cotton goods in the piece. Fig. 4 a vertical longitudinal section of the same taken on line 4—4 of Fig. 3. The machine shown in Figs. 1, and 2 55 comprises a horizontal reel 1, suitably mounted or suspended in a drying room 2, as by hangers 3, and, in the present instance, is adapted to be driven by means of a gear wheel 4, meshing with a second gear wheel 60 4<sup>a</sup>, on a driving shaft 4<sup>b</sup>. A receiving trough 5, preferably formed of galvanized wire of 1 inch mesh, is mov- 65 ably mounted beneath the horizontal reel 1, and is divided into a suitable number of receptacles or pockets by means of trans-

versely extending wire partitions 6. Ten of these receptacles or pockets are preferably formed for the purpose hereinafter described. The receiving trough 5, is adapted to rest upon and be supported by a series of friction rollers 7, suitably mounted along the floor of the drying room and adapted to receive a longitudinally extending friction-strip or plate 8, secured on the bottom of the receiving trough. The sides of the trough are provided with depending guide-strips 9, adapted to rest and slide within guide recesses 10, of a plurality of supporting standards or columns 11, arranged at either side of the receiving trough. 70 75 80

As a means for reciprocating the receiving trough during the revolution of the reel, I provide one end of the driving-shaft 4<sup>b</sup>, with a sprocket-wheel 12, carrying a sprocket chain 13, passing over a second sprocket-wheel 14, of a longitudinally extending driving-shaft 15. The driving shaft 15, is provided at its opposite end with a pulley 16, carrying a belt 17, passing over a second pulley 18. The pulley 18, is provided with a crank-arm 19, connected to an upturned end 8<sup>a</sup>, of the friction-strip or plate 8. 85 90 95

The knit goods are united or sewed together end to end into ropes 20, weighing from 100 to 125 lbs. each, and after being passed over and about the over-hanging reel 1, are united together at the ends to form endless ropes 20, so that in the revolution of the reel the goods will be allowed to accumulate as at 20<sup>a</sup>, in the pockets or receptacles 100 of the receiving trough 5, as shown. 100

When the endless ropes of goods are placed over the reel, the latter is put in motion by means of a friction-clutch 21, and the endless ropes are thus put into motion vertically by passing over the reel and falling and accumulating into pockets or receptacles below. The air in the drying room is heated at the commencement of the operation by introducing steam into the steam pipes 22, for the purpose of drying the goods, the drying room being provided with suitable ventilators (not shown) to carry off the moisture and the excess of acid gas as it develops from the heat in the heating room. 105 110 115

When the goods are almost dry, which will generally be the case after a period of from 2½ to 3 hours with a temperature of from 120 to 140° F. (this depending upon the kind and nature of the goods), the reciprocating trough 5, is put into motion by means of the friction-clutch 21, and the intermediate gearing whereby the crank-arm 19, will impart very quick and short reciprocating horizontal motions to the receiving 120 125 130 trough 5, thus causing the goods in each receptacle or pocket to be thoroughly agitated, and the attrition thus resulting, will, in the course of from 2 to 4 hours, cause the brittle superficial fuzz on the inside and outside

surfaces of the goods to be rubbed off, the detached fuzz or lint falling through the meshes of the wire body of the trough and on to the floor of the drying room, and producing on the goods a lisle-thread finish of characteristic smooth and glossy finish. A series of pins 23, carried by a longitudinally extending bar 24, in the drying room, are adapted to separate the ropes of goods while 10 in motion when passing over the horizontal reel.

The heat, while the lisleing process is going on, must be well regulated and the temperature not over 120° F. during the initial 15 operation. When the goods have been fairly well lisled, the temperature may be lowered to from 110 and 114°, but the ventilators must always be kept fully open. For heavy 20 goods the heat may be at from 120 to 124°, but it is always wise to be careful until the alkalinity of the water used is well known, as the heat and amount of acid used must depend entirely upon this property of the water used.

25 When the desired lisle-thread finish has been imparted to the goods, the heat is shut off and the room cooled down to from 90 to 100°; the goods are then taken out and placed on trucks or in baskets, and they are 30 then ready to be dyed any shade desired, or bleached as the case may be. In either case the luster of the lisle-thread finish will be permanently retained. When the goods are so lisled, it will be found that they will dye 35 much better and of a brighter shade due to the lisleing compound acting on the goods as a mordant, and the colors will be more permanently retained than when not so treated.

40 It is obvious that cotton cloth in the piece cannot be treated in the machine, such as above described for the treatment of knitted goods, and for this reason I have provided the machine illustrated in Figs. 3, and 4, of 45 the accompanying drawings. The machine is mounted in a drying room similar to the one above described for the machine for the treatment of knit goods, and comprises a pair of supporting standards 1, at either 50 end, said pairs of standards being provided at their inner sides with a plurality of horizontally extending rolls 2, provided at their ends with pinions 3, adapted to be driven by vertically mounted worm-shafts 4. The worm 55 shafts 4, are mounted in suitable bearings 5, and are provided at their upper ends with bevel gears 6, meshing with driving gears 7, carried upon a horizontally extending driving-shaft 8. The driving-shaft 8, in the 60 present instance, is supported at one end in a bearing bracket 9, and at the other in hangers 10. The driving-shaft 8, is provided with a friction-clutch 11, provided with a shifting-lever 12, whereby the clutch may be 65 thrown into operative engagement with the

driving pulley 13, to operate the driving-shaft 8, together with the rolls and intermediate gearing above described. A pair of wringer-rolls 14, are mounted on and interposed between two of the supporting standards near the top and bottom ends thereof as shown, through which the cotton cloth in full width is adapted to pass to and from the rolls 2, in the lisleing operation as now described. In the treatment of a lot of 70 goods, for example,—1000 lbs. of cotton cloth previously treated as hereinbefore described for the treatment of knit goods, one end of the cloth is sewed to the end of a piece of calico already on the machine called the 75 "dresser"; the machine is then put in motion through the friction-clutch 11, and the "dresser" carries the goods downwardly between the wringer-rolls 14, and over and about the rolls 2, in the form of endless belts 80 15, the intermediate portions of the belts 15, being in contact with each other and supported on the supporting plates 16. As the goods are carried over and between the rolls 2, and over the supporting plates 16, it is 85 90 obvious that the intermediate or rubbing portions of the endless belt portions 15, of the cloth will be subjected to great attrition adapted to rub and break off the superficial fiber or fuzz, rendered brittle by the action 95 of the chemicals in the lisleing compound, and a very superior lisle-thread finish of great luster and gloss is imparted to the goods.

It will be understood that in starting the 100 machine as above described that the end of the goods first sewed to one end of the "dresser" will be unsewed when the "dresser" has been run out of the machine 105 at the top by the goods taking the place of the "dresser" and the adjacent ends of the goods are then sewed together to make an endless piece of the whole lot, and this endless piece is kept in the machine for a period of about 2 hours, the machine being 110 reversed at intervals of an hour or half hour whereby the goods will be caused to run in an opposite direction, thus greatly facilitating the lisleing operation.

When the desired finish has been imparted 115 to the goods, I open the two sewed ends of the goods and sew to one end of the "dresser" hereinbefore referred to, which starts the machine which causes the other end of the goods to be carried out of the machine, and 120 as the goods are carried out they are conveyed into a basket or truck or rolled on a roll preparatory to be given the finishing dye bath or bleach treatment as desired. The temperature in the room should be similar 125 to that described for the drying room containing the machine for the treatment of knit goods. If a light gray color is to be produced on the goods, I add to the solution a little iron sulfate in the proportion of 130

from  $\frac{1}{2}$  to 1% of the weight of the compound. After the goods have been given the desired preliminary finish, I wash the same in water to which has been added from 1 to 2% of 5 sumac or of tannic or of gallic acids; this causes the formation of a light gray iron tannate which is a fast color.

Having thus described my invention, what I claim and desire to secure by Letters Patent is,—

1. The process of giving lisle-thread finish to vegetable fabrics, consisting in (1) boiling the goods sufficiently long to render the same absorbent, (2) hydro-extracting, (3) 15 placing in a carbonizing solution from 15 to 20 minutes, (4) hydro-extracting so as to retain carbonizing liquor equal to 50 to 60% of the dry weight of the goods, (5) and finally subjecting to heat and attrition until 20 the filamental fuzz is removed and a lisle-thread finish imparted to the goods.
2. The process of giving lisle-thread finish to vegetable fabrics, consisting in (1) boiling the goods to render the same absorbent, (2) washing and hydro-extracting, (3) 25 saturating with a carbonizing solution containing alum, starch, and hydrochloric acid (4) hydro-extracting the surplus liquor (5) and finally subjecting to heat and attrition 30 until a lisle-thread finish is imparted to the goods.
3. The process of giving lisle-thread finish to vegetable fabrics, consisting in (1) boiling the goods, (2) hydro-extracting, (3) 35 saturating in a carbonizing solution containing alum, starch, hydrochloric acid and iron sulfate (4) hydro-extracting, leaving carbonizing solution equal to from 50 to 60% of the dry weight of the goods, (5) and finally 40 subjecting to heat and attrition until the desired lisle-thread finish has been imparted to the goods.
4. The process of lisleing and dyeing vegetable fabrics, consisting in (1) boiling and 45 washing to render the same absorbent, (2) hydro-extracting, (3) impregnating the fabric with a chemical solution containing an acid radical adapted to carbonize the superficial filamental fuzz when subjected to heat 50 and a metallic mordant adapted to the color desired, (4) hydro-extracting, leaving solution therein equal to from 50 to 60% of the dry weight of the goods, (5) subjecting to heat and attrition at a temperature of from 55 110 to 120° F. until the superficial filamental fuzz has been removed and the surface finished, (6) subjecting to a neutralizing reacting and fixing solution, and (7) hydro-extracting.

5. The process of lisleing and dyeing vegetable fabrics, consisting in (1) boiling and washing, (2) hydro-extracting (3) saturating with a carbonizing solution containing alum, starch and hydrochloric acid, (4) hydro-extracting a portion of said liquor, (5) subjecting to heat and attrition at a temperature of from 110° to 120° F. for from two to three hours until the desired lisle-thread finish has been obtained, (6) subjecting to a neutralizing dyeing and fixing solution, (7) washing, (8) hydro-extracting and drying.

6. The process of lisleing and dyeing vegetable fabrics, consisting in (1) boiling, (2) hydro-extracting, (3) saturating with a carbonizing solution having a metallic mordant adapted when subjected to the neutralizing, reacting and dyeing solution to impart the color desired, (4) hydro-extracting, (5) subjecting to heat and attrition until the superficial fuzz has been removed and the surface finished, and (6) subjecting to a neutralizing, reacting and dyeing solution.

7. The process of treating vegetable fabrics, consisting in (1) boiling in an alkali bath and washing whereby the same are rendered chemically absorbent, (2) hydro-extracting, (3) saturating with a chemical solution containing an acid radical and a mordant adapted, respectively, to carbonize the superficial filamental fuzz and impart the color desired when subjected to the action of the dyeing agent, (4) hydro-extracting, (5) subjecting to heat and attrition, and (6) subjecting to a solution containing a neutralizing reacting and dyeing agent.

8. The process of treating vegetable fabrics, consisting in (1) boiling and washing to render the same absorbent, (2) hydro-extracting, (3) saturating with a solution containing a metallic mordant adapted to impart the color desired and an acid radical adapted when subjected to the neutralizing dyeing and fixing solution to carbonize the fuzz when exposed to heat, (4) hydro-extracting so as to retain solution equal to from 50% to 60% of the dry weight of the goods, (5) subjecting to heat and attrition at 110° to 120° F., (6) subjecting to a neutralizing dyeing and fixing solution, (7) 100 washing, and (8) hydro-extracting and drying.

In testimony whereof I have affixed my signature, in presence of two witnesses.

ALEXANDER N. DUBOIS.

Witnesses:

KUNC B. SCHOTTE,  
JOHN T. DAVIS.